

## UNITED STATES PATENT OFFICE.

ERNST FRIEDERICH, OF BERLIN-CHARLOTTENBURG, GERMANY, ASSIGNOR TO RADIO CORPORATION OF AMERICA, A CORPORATION OF DELAWARE.

## GLOW CATHODE AND ELECTRON TUBE CONTAINING SAME.

No Drawing. Application filed November 28, 1925, Serial No. 72,044, and in Germany December 1, 1924.

My invention refers to electron tubes and more especially to the glow cathodes forming part of such tubes. It is an object of my invention to provide a cathode and a tube embodying such cathode which is more efficient than similar articles hitherto used.

In the glow cathode forming part of electron tubes tungsten wire and wires of other metals have been used which contain additions of oxides having a high melting point. By such addition the emission of electrons is increased far beyond the emission taking place in the case of pure metal wire. It is also known to still further increase the efficiency of glow cathodes containing such additions by subjecting them to a treatment of reduction with metals of an alkali or an alkaline earth or with carbon. It is this latter method which has been practiced on a large scale; however, the treatment with carbon entails the drawback that the tungsten wire combines with the carbon to form a carbide, whereby it loses its elasticity and gets brittle. The chances of these wires breaking during transport or during the use of these tubes are very great.

It has now been ascertained that if the pure tungsten wire is enveloped in a skin or coating of thorium carbide, an extraordinarily favorable emission of electrons is obtained, which is even superior to the emission obtained with tungsten wire containing thorium oxide which has been subjected to reducing treatment. This fact could not be foreseen as it could not be assumed that thorium carbide would have the same electron emission as metallic thorium. It has now been ascertained by extensive investigation that this is the fact.

The glow cathode according to this invention is a metal wire, for instance a tungsten wire, capable of high electron emission and which is provided with a skin or coating containing a carbide. My invention further relates to the method of producing such cathodes and the tubes of which they form part.

In the production of cathodes according to this invention I have found it particularly useful to employ a mixture of  $\text{ThO}_2 + 4\text{C}$ , using as a binder a solution of acetylic cellulose in an organic solvent. It is an easy matter to coat a wire several hundred meters long with a coating consisting of such mixture, the coating procedure being well known so as not to require further descrip-

tion. The manufacture of the tubes by means of a wire coated in this manner is practiced in a well known manner, the carbonization of the binder and the formation of the carbide taking place in the usual course of operations without any special treatment being required. The binder is carbonized when heating the wire under the action of the vacuum pump to about 400° C. and the carbide forms in the mixture remaining on the surface of the wire when the tube is supplied with current, which can be done either when it is still connected with the vacuum pump, or also after the melting off. Tubes manufactured in this way furnish already at low temperature an emission equal to that of a wire having the same surface, but lacking the coating, but such tubes enjoy a very long life and all danger of breaking of the wire is done away with inasmuch as the tungsten wire itself carrying the skin or coating does not contain any carbon.

As a rule tungsten wire coated with thorium carbide has proved to be useful. I have, however, ascertained that also other carbides can be used with advantage, for instance the carbides of the metals of the second, third and fourth groups of the periodical system of elements, which are known to have a high electron emitting capacity, and also the carbides of the rare earths. In these cases it can be proved advantageous to replace the tungsten by another metal acting as carrier, for instance a noble metal such as platinum.

As a rule pure metals will be used as carriers for the carbides. It may, however, happen sometimes that the carbide coating is prematurely removed in some place either from mechanical causes or by evaporation in consequence of overloading, so that in consequence of a different emission of electrons or different radiation there arise differences of temperature whereby single places are overloaded and cause the cathode to burn through prematurely. In order to avoid this as far as possible I have found it useful to employ a carrier wire which already contains a small quantity of carbon, as a rule not exceeding 0.1 percent. I hereby prevent the difference in the emission of electrons from becoming too great and I prevent the wire from burning through.

I wish it to be understood that I do not

desire to be limited to the exact substances, proportions, temperatures and operations described, for obvious modifications will occur to a person skilled in the art.

5 1. I claim:—

1. A glow cathode for electron tubes comprising a metal wire containing a small percentage of carbon and a coating on this wire containing a carbide of a metal capable of 10 high electron emission.

2. A glow cathode for electron tubes comprising a wire of tungsten containing a small percentage of carbon and a coating on this wire containing thorium carbide.

15 3. A cathode for electron tubes comprising a wire of tungsten containing a small quantity of carbon not exceeding 0.1 percent and a skin or coating on this wire containing thorium carbide.

20 4. The method of forming a cathode which

consists in coating a highly refractory filamentary core with a mixture of carbon and a compound of a metal having a high electron emitting capacity and heating the resulting product sufficient to form a carbide 25 of the metal.

5. The method of forming a cathode which consists in coating a refractory core with a mixture of thorium oxide and carbon and heating the resultant product until a coating 30 of thorium carbide is formed on the core.

6. The method of coating a filamentary cathode which consists in applying to the surface thereof a mixture of thorium oxide, carbon and a binder, and heating the cathode to decompose the binder, reduce the thorium oxide and form a film of thorium carbide on the surface of the cathode. 35

In testimony whereof I affix my signature.  
ERNST FRIEDERICH.